

# UNITED STATES PATENT OFFICE.

ROBERT PERCY BROUSSON, OF LONDON, ENGLAND.

## MANUFACTURE OF GAS.

1,313,514.

Specification of Letters Patent.

Patented Aug. 19, 1919.

No Drawing.

Application filed September 28, 1915. Serial No. 53,151.

To all whom it may concern:

Be it known that I, ROBERT PERCY BROUSSON, a subject of the King of Great Britain and Ireland, residing at London, England, 5 have invented Improvements Relating to the Manufacture of Gas, of which the following is a specification.

The enrichment of ordinary coal gas by the use of cannel coal is very expensive owing to the small quantity of cannel coal that is now available and its consequent high price and to the fact that the coke from cannel coal does not find a ready market. It has become usual, in gas works of any 15 considerable size, to dispense with the use of cannel coal or substitutes like natural asphalts and to install apparatus for the production of carbureted water gas whereby the coal gas can be enriched and, when desired, the output of gas increased to meet the demand, but, as such apparatus involves considerable outlay and the employment of men skilled in its manipulation, many small 20 gas works have not adopted it.

25 The object of the present invention is to enable the output of gas to be increased or enriched, or both, more economically than is possible with either of the above methods and without the use of special machinery or plant, for instance such as is 30 needed in the production of carbureted water gas.

Now according to my invention I intimately mix bitumen obtained from distillation with coal in suitable proportions and treat the mixture in retorts in the way coal is ordinarily treated whereby I obtain a greater output of gas than can be obtained from a corresponding amount of coal alone 40 and even from corresponding amounts of coal and bitumen treated separately in retorts.

In this way the output can be largely increased with a comparatively small addition to the amount of material carbonized, or the output required, enriched if necessary can be obtained with a considerable reduction in the amount of material carbonized, it may be even to such an extent that 50 the number of retort settings in use can be decreased.

Bitumen derived from distillation differs from natural bitumen in that the percentage of ash or foreign matter is very 55 small; that a small proportion in admixture with coal largely increases the yield

or quality of gas, and that the coke is not detrimentally affected by its use.

The bitumen I prefer is produced by carrying the normal petroleum distillation 60 process to a further stage than is usual for the production of bitumen viz. to about 750° F. or to such a temperature as will produce a bitumen which, on cooling, becomes a hard black mass that is brittle or 65 capable of being readily broken, or even ground, and is refractory in the sense that the temperature required to complete the carbonization of the bitumen in the retorts, though probably somewhat lower, will approach more or less closely that required 70 to complete the carbonization of the coal; however since, weight for weight, the bitumen contains more volatile matter than the coal, it will naturally give off gases more 75 rapidly in the primary stages of carbonization of the intimate mixture of bitumen and coal, but both materials will reach the condition of coke at substantially the same time gas being evolved from both materials 80 until that condition is reached at the end of the process.

The invention can be carried out in a very simple manner, the desired proportion of bitumen, reduced, if need be to the required size, being thoroughly mixed with the coal to be carbonized, the mixture being made before charging into the retorts or in the retorts and the gas making conducted in the usual way, care being taken 85 that the temperature of carbonization is not too low.

The proportion of bitumen may be varied according to particular requirements and qualities of coal used. I have found 95 that with charges comprising 95 per cent. of good quality coal and 5 per cent. of bitumen, the output of gas per ton was considerably increased, the candle power or calorific value being maintained the same, 100 the output of gas from the coal and bitumen mixture showing an increase of over two thousand cubic feet per ton as compared with the average output per ton of coal alone; with a mixture of 92½ per cent. of 105 coal and 7½ per cent. of bitumen there was obtained an increase of over five thousand cubic feet per ton as compared with the average output per ton of coal. The yield of gas obtained from the mixture is considerably more than the yield of gas from 110 corresponding amounts of coal and bitumen

carbonized separately. Although higher percentages of bitumen may possibly be used with advantage, my experiments indicate that high percentages of bitumen will 5 not give correspondingly high yields of gas; moreover it should be borne in mind that with high percentages of bitumen difficulties may occur, such as excessive flame or flare during charging and deposit of liquid 10 bitumen at the cooler ends of retorts of the horizontal type.

In cases where it is desired that the illuminating power or the calorific value of the gas shall be high for the quality of coal 15 used, the conditions under which the mixture of coal and bitumen is carbonized are regulated in a similar manner to that usual in the manufacture of gas from coal when a rich gas or a gas of high calorific value is 20 required.

The invention renders available to gas makers a method of enriching or increasing the output of an ordinary coal gas works which is cheap, simple and effective and is 25 capable of increasing the output to meet a sudden demand due to fog or other cause much more quickly than can be done with carbureted water gas plant which takes a considerable time to get under way. Furthermore, the coke resulting from carbonization of the mixture is of good physical 30 quality and produces less clinker than ordinary coke when burnt in furnaces.

The cost of the bitumen referred to 35 delivered at the works should not be excessive owing to low transport costs and in the works it can be largely handled in the same way, by the same men and machinery and submitted to the same treatment as the coal 40 so that the process of gas making is not complicated by its use.

What I claim is:—

1. A process of manufacturing gas consisting in intimately mixing with coal bitumen of a hard, brittle, stable and refractory nature obtained by distillation of petroleum at approximately 750° F., and subjecting the mixture in the retorts to the heat treatment usual in coal gas manufacture, substantially 50 as described.

2. A process of manufacturing gas consisting in intimately mixing with coal bitumen of a hard, brittle, stable and refractory nature obtained by the distillation of petroleum at approximately 750° F., and subjecting the mixture in the retorts to the heat treatment usual in coal gas manufacture, substantially as described.

3. A process of manufacturing gas con-

sisting in intimately mixing with coal a 60 bitumen of a hard, brittle, stable and refractory nature obtained by distillation, said bitumen requiring to complete its vaporization a temperature closely approaching the temperature required to complete the vaporization of the coal, and subjecting the mixture in the retorts to the heat treatment usual in coal gas manufacture, substantially as described.

4. The process of manufacturing gas, consisting in mixing with coal a relatively small quantity of finely divided bitumen of a hard, brittle, stable and refractory nature requiring to complete its carbonization a 65 temperature approaching closely the temperature required to complete the carbonization of coal, thoroughly mixing the divided bitumen with the coal, whereby the bitumen will be evenly distributed throughout the mass, and then subjecting the mixed bitumen and coal to a high carbonizing heat in a retort.

5. The process of manufacturing gas consisting in first obtaining bitumen of a hard, brittle, stable and refractory nature by distilling petroleum to a final temperature of approximately 750° F., finely dividing said hard brittle bitumen, thoroughly mixing the divided bitumen with coal to evenly distribute it throughout the mass, and then subjecting the mixed bitumen and coal to the heat treatment usual in coal-gas manufacture, whereby the bitumen and coal will be 80 carbonized simultaneously and the resulting gases thoroughly mixed in the retort 85 during the process of carbonization.

6. The process of manufacturing gas consisting in first producing a hard brittle bitumen by distilling petroleum to a final temperature of approximately 750° F., whereby 90 the said bitumen will require in its carbonization approximately the same degree of heat required to complete the carbonization of coal in the manufacture of gas, mixing said hard brittle bitumen with coal, and then 95 subjecting the mixed bitumen and coal to a temperature sufficient to carbonize the coal, whereby the mixed bitumen and coal will be progressively carbonized in substantially the same proportions and the resulting gases 100 will be thoroughly mixed in the retort throughout the period of carbonization.

Signed at 75/77 Cornhill London England this eleventh day of September 1915.

ROBERT PERCY BROUSSON.

Witnesses:

P. E. MATTOCKS,  
F. C. SMITH.